

Patented June 22, 1926.

1,589,636

## UNITED STATES PATENT OFFICE.

JULIUS H. GILLIS, OF ELIZABETH, NEW JERSEY, ASSIGNOR, BY MESNE ASSIGNMENTS, TO ANACONDA SALES COMPANY, A CORPORATION OF DELAWARE.

### PROCESS OF MAKING ROOFING ELEMENTS.

No Drawing.

Application filed July 23, 1923. Serial No. 653,386.

This invention relates to the manufacture of roofing elements in the form of boards, strips, shingles, tiles, and the like, and especially elements which consist of a base of the type commonly used in so-called asphalt shingles having a protective metallic covering applied to the weather surface of the base.

Elements of the type referred to are shown and described in Letters Patent No. 1,449,058, issued March 20, 1923, to Thomas Robinson, and also in a somewhat modified form in an application of Robinson filed February 10, 1923, bearing the Ser. No. 618,246.

The ordinary asphalt shingles now in general use are satisfactory for many purposes but they involve a disadvantage due to the fact that when laid in place on the roof and exposed to the weather they have a tendency to warp or curl. Also continued exposure to the sun produces deterioration due to the volatilization of the oils contained therein. Shingles made wholly of metal overcome the disadvantages pointed out and have an attractive appearance, especially when made of metal such as copper, which lends itself to the production of various color effects. These metal shingles, however, transmit heat with great rapidity and it is necessary to provide sheathing which acts as a heat insulator.

The composite shingles disclosed in the Letters Patent and in the application combine the several advantages of the two types, inasmuch as the metal coating adds to the life of the element by resisting wear and by preventing deterioration. Also the shingle which has a metallic coating only on its exposed or weather surface has an appearance similar in general to a solid metal shingle, and since a comparatively thin coating is used, applied only to a portion of the shingle surface, the cost of these elements is relatively low and they may be handled and laid quite as easily as the ordinary asphalt shingles uncoated.

In manufacturing the coated elements referred to the base used is made by well-known methods and the individual shingles are cut to the desired size and shape prior to the coating operation. This metallic coating is then applied in various ways and

one convenient method is by electro-deposition. In the latter process it is necessary, owing to the fact that the base is an insulator, to provide a conducting layer so that the electro-deposition may be carried on, and the present invention is directed to a process for applying a metallic coating by electro-deposition, including the steps incidental to applying the conducting coating over which the metal is to be deposited.

In carrying out the new process the base is first treated with an adhesive and a conducting material, usually in powdered form, is applied to the base while the surface is still tacky. The base so coated is then supported in a convenient manner in an electrolytic tank and the metal deposited over the conducting layer in the usual manner.

The application of the conducting coating involves several essentials; for instance, the adhesive used must be relatively inexpensive, must be easily applied in a thin film and must be capable of being applied rapidly in such a way as to completely cover the conducting surface. If this film does not cover all parts of the surface of the base over which the metallic layer is to be applied, the metal coating will be interrupted and the element so formed will be imperfect and unacceptable for use. Again, the adhesive must be quick-drying so that this step in the process will not consume a large amount of time, and also the adhesive must be of such a character that it will bind the conducting layer firmly in place so that the element so treated is capable of standing the handling incidental to the electrolytic process. It is also necessary that the adhesive should be unaffected by the electrolyte while the deposition is taking place, and although there are numerous adhesives which fulfill all other requirements yet if these adhesives dissolve in the electrolyte they render the liquid impure and in many cases result in slimes which interfere with the deposition.

I have found that an adhesive which fulfills all the requirements above, may be made by dissolving asphalt in carbon tetrachloride. The carbon tetrachloride used is the ordinary commercial product and asphalt is dissolved in it until there is formed a substantially saturated solution. Asphalt is not highly soluble in this liquid but sufficient

may be dissolved to produce the desired adhesive material.

In treating roofing elements for the purpose of placing them in condition for the deposition of the metal, the elements as produced are conveyed to a treating tank which contains the substantially saturated solution of carbon tetrachloride above described, and this liquid is applied over the surface of each element by brushing. While it is equally possible to use spraying or even dipping, experience has indicated that brushing is the most satisfactory method and the workman will apply a thin coating of the adhesive material to that portion of the surface of the element upon which the metal is to be deposited. As will be seen later, the adhesive need not be carefully limited to the exact area which is to carry the metallic layer, but the workman will ordinarily confine the adhesive coating as closely as possible to this area in order to save time and also to save the adhesive.

The coated elements are then conveyed to a heating chamber which is exhausted by suitable fans so that in drying the carbon tetrachloride may be recovered. The application of heat in this chamber not only hastens the evaporation but also serves to keep the residual asphalt in a tacky condition.

When this step in the process is completed the elements are conveyed to another station where the conducting material is applied. Various substances may be used for this purpose but it has been found that powdered graphite is the most satisfactory. It is inexpensive, forms a good conductor, and the particles may be applied and spread so as to form a thin coating without abrading the surface of the asphalt. For this purpose a quantity of graphite is placed on the shingle, sufficient to form the coating and the graphite is then spread over the surface by soft brushes. This operation can be carried on quite rapidly and it is comparatively easy to produce a thin, even, and continuous film of graphite which adheres firmly to the tacky asphalt. While other materials, such as powdered metal, may be applied, and will serve the purpose equally well in some respects, it will be recalled that graphite has certain lubricating qualities which make it preferable, inasmuch as the particles of powdered metal are usually sharp so that they would cut or abrade the asphalt layer during the brushing operation.

The elements so coated are now conveyed to the electrolytic tanks and are ordinarily mounted in suitable clamps which serve to expose only that portion upon which the deposition is to take place. These clamps may be in various forms but are made of non-conducting material so that they are not

affected by the electrolyte and so that deposition will not take place upon them, although they are beneath the surface of the liquid in the tanks. By using a clamp which exactly defines the metallic layer it is possible to apply the adhesive and the conducting material without paying strict attention to the limits of the area. In fact in some instances it is possible to apply the adhesive by dipping and the saving of time by such an operation will compensate for the loss of material to a great extent. The elements are left in the electrolytic troughs until a coating of the desired thickness has been deposited thereon, whereupon they are removed and, after drying, may be subjected to a treatment for changing the color of the metal by any of the well-known processes.

The use of carbon tetrachloride as a solvent makes it possible to use asphalt as the adhesive material, and accordingly, since the base itself contains asphaltic compositions, this adhesive layer, when subjected to the heat treatment, forms a layer which is homogeneous with the base and does not separate from the base upon exposure of the element to the weather. The asphalt solution may, however, be applied with equally satisfactory results to any of the well-known materials used for the base, and since this ingredient is relatively inexpensive and the carbon tetrachloride is almost completely recovered during the process it will be seen that this step in the process involves but little expense. The graphite is also relatively inexpensive, inasmuch as one pound will serve to cover an area of approximately 140 to 150 square feet. The application of the adhesive may be carried on by ordinary workmen, since no high degree of skill or attention is required.

I claim:

1. A process for the manufacture of roofing elements which comprises applying to the surface of a base impregnated with a waterproofing compound a solution of the waterproofing compound in a volatile solvent, applying thereto a conducting material, and electrodepositing a metallic coating over the conducting material.

2. A process for the manufacture of roofing elements which comprises applying to the surface of a base impregnated with an asphaltic compound, a solution of this compound in a volatile solvent, applying thereto a conducting material, and electrodepositing a metallic coating thereover.

3. A process for the manufacture of roofing elements which comprises applying to a base impregnated with an asphaltic material a substantially saturated solution of this asphaltic material in a volatile organic solvent, partially evaporating the solvent, applying a conducting material to the base

while the surface thereof is still tacky, and electro-depositing a metallic coating thereover.

4. A process of the manufacture of roofing elements which comprises applying to a base impregnated with an asphaltic material a solution of this asphaltic material in

carbon tetrachloride, evaporating the carbon tetrachloride, applying a non-abrasive conducting material to the base while the surface thereof is still tacky and electro-depositing a metallic coating thereover. 10

In testimony whereof I affix my signature.

JULIUS H GILLIS.